# EUROPEAN PATENT APPLICATION

(11) **EP 2 014 825 A1**
(43) Date of publication of application: **14.01.2009**
(21) Application number: 08104655.9
(22) Date of filing: 07.07.2008
(51) Int. Cl.: D06N 7/00, D06M 23/14, A41D 13/12, D06N 3/00, D04H 1/46

(54) **Coated cloths and methods for manufacturing the same**

(30) Priority: 10.07.2007 CN 200710129415
(71) Applicant: Winner Industries (Shenzhen) Co., Ltd., Longha Shenzhen 518109 (CN)
(72) Inventor: LI, Jianquan Winner Industries (Shenzhen) Co., Ltd., 518109, Shenzhen City (CN)
(74) Representative: CAPRI

(57) **Abstract**

Disclosed are coated cloths wherein the coating that is waterproof and breathable is crosslinked to the fabric and methods for manufacturing the same. The coated cloth provided can be used to manufacture medical gowns or drapes to prevent people in operation from being cross-infected.

## Description

### Cross Reference to Related Applications

This application claims the benefit of Chinese Patent Application No. 200710129415.9 filed July 10, 2007 which is incorporated herein by reference in its entirety.

### Technical Field

This invention is directed to cloths and particularly to coated cloths.

### Background of the Invention

Conventional medical cloths including surgical gowns and drapes are generally manufactured with a non-woven fabric that people feel compact, soft and non-irritating. However, the conventional medical cloths normally are not waterproof. As such, during operation, blood or a body fluid of a patient may soak the surgical gowns and drapes, which will possibly make the people in operation cross-infected.

### Summary of the Invention

To address the problem in the art, there is provided a cloth comprising a fabric and a coating provided on at least one part of the fabric. The coating is waterproof and breathable and is crosslinked to the fabric to prevent the coated part of the fabric from soaking by a liquid.

In another aspect, there is provided a method for manufacturing a cloth including: providing a fabric; coating at least one part of the fabric with a waterproof and breathable coating; and subjecting the coated fabric to a high temperature such that the coating can be crosslinked to the fabric.

The cloth provided herein can prevent a liquid such as water, alcohol, blood and oil from soaking. Therefore, the cloth can be used for a disposable protective clothing and its accessories such as insulation garments, experimental clothing, protective hats, shoe covers and oversleeves, and household protective articles such as bed sheets, pillowcases, tablecloths, and spread sheets.

In some embodiments, the cloth provided herein is used to make medical articles such as surgical gowns and drapes which can protect the people in operation from the cross infection.

### Brief Description of the Drawing

Figure 1 is a schematic diagram illustrating a cloth according to an embodiment of the present invention; and

Figure 2 is a schematic diagram illustrating a cloth according to another embodiment of the present invention.

### Detailed Description of the Invention

Fig. 1 is a schematic diagram illustrating a cloth according to an embodiment of the present invention. The cloth has a fabric 1 and a coating 2 provided on one side of the fabric 1.

Fig. 2 shows a cloth according to another embodiment. Coatings 2 and 3 are provided on both sides of the fabric 1.

] The fabric 1 is normally, but not be limited, a spunlaced non-woven fabric which can be made of cotton or a mixture of cotton and a polymer which is well known for artisan in the art such as polypropylene or polyester fiber or a mixture thereof. Preferably, the fabric 1 is made of cotton which is comfortable and nonirritating.

The coating 2 and coating 3 that should be waterproof and breathable, can be the same or different and selected from one of those coatings that are conventionally used in the art, for example, polytetrafluoroethylene cotaings, polyurethane coatings, acrylate coatings or a combination thereof. In some embodiments, the coating is polytetrafluoroethylene coatings or polyurethane coatings. In this embodiment, the coating is a polyurethane coating.

The cloth provided herein can be used to manufacture different articles such as surgical gowns and coated surgical drapes.

A method for preparing the cloth as provided herein comprises coating a fabric with a coating on at least one part of the fabric; and subjecting the coated fabric to a high temperature such that the coating is cross-linked to fiber of the fabric.

The coating step in the method can be performed by a rotary-screen-printing coating, a roll-coating, a flow-coating, a foam-coating, a spray-coating, a blade-coating, a transfer-coating or a combination thereof.

The coated fabric can then be dried by any one of radiation, blast-heating and cylinder-drying processes or a combination thereof. Afterwards, the dried coated fabric is treated at a high temperature which is normally ranging from 100° to 200°C (the range of temperature is depend on the specific material of the fabric) to make the coating cross-linked with fiber of the coated fabric. This process can be performed by a heated blast.

Where the fabric is a spunlaced non-woven fabric that is made of cotton and a polymer i.e, polypropylene or polyester fiber, a ratio between cotton and the polymer may be 65%-95%:35%-5%. Compared to a spunlaced non-woven fabric made of cotton, a spunlaced non-woven fabric with cotton and a polymer has advantages of a lower cost and a better anti-crease performance.

General concepts and various embodiments of the present invention have been disclosed above. Without departing from the spirit of the present invention, modifications, substitutions and improvements can be made for those skilled in the art, which should be within the scope of the present invention.

## Claims

1. A cloth comprising a fabric and a coating provided on at least one part of the fabric, wherein the coating that is waterproof and breathable is crosslinked to the fabric such that the part of fabric can prevent a liquid from soaking.

2. The cloth of claim 1, wherein the coating is selected from the group consisting of a polytetrafluoroethylene coating, a polyurethane coating, an acrylate coating and a combination thereof.

3. The cloth of claim 2, wherein the fabric is a spunlaced non-woven fabric.

4. The cloth of claim 3, wherein the spunlaced non-woven fabric is made of cotton or cotton and a polymer.

5. The cloth of claim 4, wherein the spunlaced non-woven fabric is made of cotton and a polymer and a ratio between cotton and the polymer is 65%-95%:35%-5%.

6. The cloth of claim 1, wherein the cloth is used for manufacturing a medical gown or drape.

7. A method for manufacturing a cloth, comprising:
a) providing a fabric;
b) coating a waterproof and breathable coating on at least one part of the fabric; and
c) subjecting the coated fabric to a high temperature such that the coating is crosslinked to the fabric.

8. The method of Claim 6, wherein step c) is performed by a heated blast having a temperature ranging from 100° to 200°C.

9. The method of claim 7, wherein the step b) is performed by a rotary-screen-printing coating, a roll-coating, a flow-coating, a foam-coating, a spray-coating, a blade-coating or a transfer-coating.
